

1

3,332,835

**PROCESS OF FORMING WOOD-FIBER INSULATION BOARD CONTAINING SULFINE POLYMER, ALDEHYDE AND MINERAL ACID AND BOARD THEREOF**

Keith L. Smith, Charleston, W. Va., assignor to Union Carbide Corporation, a corporation of New York  
No Drawing. Filed Jan. 29, 1964, Ser. No. 341,112  
11 Claims. (Cl. 162—168)

This invention relates to the production of wood-base construction and insulation board from wood-fiber pulp. More particularly, the invention relates to the incorporation in such board of minor amounts of certain substantially water-soluble sulfine polymers, alone or in combination with suitable aldehydes, or mixtures of such aldehydes and mineral acids, whereby enhanced dry- and wet-strength, improved stiffness, and other desirable physical properties are obtained. The invention further comprehends the improved construction and insulation board produced in this manner.

Wood-fiber board is widely used as a construction material and is at present the most common low cost rigid insulation for general construction use. It is used in the form of panels ranging in thickness up to about an inch for rigid interior wall insulation, as interior acoustical surfacing for ceilings, and, with a suitable surface coating, for wall sheathing. Processes used to produce such board are similar to the conventional paper forming process. Virgin or reclaimed groundwood is generally used and the wood-pulp spread on a screen or wire with dewatering being accomplished by gravity and by suction below the wire. The board is then squeezed or pressed by any of a variety of techniques, cut into panels of suitable size, and dried in an oven at an elevated temperature, generally from about 200 to 350° F.

The physical properties of commercial wood-fiber board are typically a result of a compromise between the conflicting requirements of insulation properties, tensile properties and cost. Since wood-fiber board, in common with paper products generally, retains only a small fraction of its dry strength when soaked in water the tensile strength and stiffness under conditions of high humidity or water saturation are of critical concern. Stiffness assumes special importance where the material is used for ceiling tile or composite roof deck-ceiling because of the tendency for sagging and warping to occur after prolonged periods of exposure to relatively high humidity levels. Heretofore, improvement in wood-fiber board properties has been achieved either by subjecting the pulp slurry to prolonged beating or by the addition of starch in amounts of up to 3 to 4 percent. However, the former is unsatisfactory because of increased costs, decreased production rate as a result of increased water retention, and improvement in tensile properties only at the expense of a substantial increase in density and consequent reduction in insulation value; while the latter is undesirable because of the tendency for starch addition to substantially increase the drain time and water retention in the board on the wire and thereby decrease production rate and also because the board retains a pronounced susceptibility to moisture.

It is a primary object of this invention to provide an improved wood-fiber board having enhanced dry tensile strength, wet tensile strength, initial stiffness and apparent stiffness after continued exposure to high-moisture conditions. A further object of this invention is to provide an improved process for the production of wood-base construction and insulation board wherein the addition of minor amounts of additives provides enhanced tensile and other physical properties. A still further object of this

2

invention is to provide additives to wood-fiber pulp which permit production of wood-fiber board at a faster rate, with less water retention at various stages in the manufacturing process, thereby reducing production cost and increasing the production capacity of board manufacturing equipment. Yet another object of the invention is to provide additives for wood-fiber board manufacture which greatly improve the physical properties of the wood-fiber board at low levels of add-on. Other objects and advantages of the invention will be apparent from consideration of the following detailed description together with the appended claims.

It has now been found that the disadvantages of the prior art methods of producing wood-base construction and insulation board, as hereinabove described, can be substantially overcome and a greatly improved board produced through the practice of the present invention which comprises applying to the wood-fiber pulp from which said board is formed a strength improving composition comprising a water-soluble polymer of an alpha-ethylenically unsaturated sulfine, i.e. a sulfonium compound possessing a terminal ethylenic unsaturation. While addition of said polymer alone results in a substantially improved product, even greater improvement in the physical properties of wood-fiber board can be achieved by applying, in combination with such polymer, a minor amount of an aldehyde or, more preferably, a mixture of an aldehyde and a mineral acid as hereinafter described; and, accordingly, addition of said aldehyde or mixture of aldehyde and mineral acid is preferred in the practice of this invention.

Specifically, the sulfine polymers contemplated by this invention as treating agents for wood-fiber board include the homopolymers of the alpha-ethylenically unsaturated sulfines represented by the formula:



wherein R designates either a hydrogen atom or a methyl radical; R' designates an alkylene radical containing from 1 to about 4 carbon atoms and preferably from 2 to 3 carbon atoms, such radical more preferably separating the adjacent (in this instance oxygen and sulfur) atoms by a carbon chain containing at least 2 carbon atoms; and R'' designates a lower alkyl radical containing from 1 to about 4 carbon atoms and preferably from 1 to 2 carbon atoms. As illustrative of such ethylenically unsaturated sulfines, there can be mentioned: acryloxy-methyldimethylsulfonium methyl sulfate, (2-acryloxyethylmethyl)disulfonium methylsulfate, (2 - acryloxyethyl) methylbutylsulfonium methylsulfate, (2 - acryloxyethyl) methylbutylsulfonium methylsulfate, (4-acryloxybutyl)dimethylsulfonium methylsulfate, (2 - methacryloxyethyl) dimethylsulfonium methylsulfate, and the like.

The polymeric treating agents of this invention also include interpolymers (i.e., copolymers, terpolymers and quadripolymers, etc.) of the aforementioned sulfines, especially with at least one other copolymerizable monomer as, for instance, the alkylthioalkyl acrylates and methacrylates represented by the formula:



wherein R, R' and R'' are as defined above, such as methylthiomethyl acrylate, methylthioethyl acrylate, ethylthioethyl acrylate, butylthioethyl acrylate, methylthiobutyl acrylate, methylthioethyl methacrylate, and the like; acrylamide and lower alkyl substituted acrylamides, such as methacrylamide and N,N-dimethylacrylamide; the vinyl-

benzenes, including vinylbenzene and lower alkyl substituted vinylbenzenes, the alkyl and cyanoalkyl acrylates and methacrylates represented by the formula:

III



wherein R is as defined above, R''' designates an alkylene radical containing from 1 to about 10 carbon atoms and preferably from 1 to 4 carbon atoms, and Y designates either a hydrogen atom or a cyano (—CN) radical, such as methyl acrylate, ethyl acrylate, butyl acrylate, 2-ethylhexyl acrylate, methyl methacrylate, 2-cyanoethyl acrylate, and the like; the vinyl alkanoates represented by the formula:

IV



wherein R'' is as defined above, such as vinyl acetate, vinyl propionate, vinyl butyrate, vinyl pentanoate, and the like: the N-alkyl-N-vinylamides represented by the formula:



wherein each R'' is independently selected as defined above, such as N-methyl-N-vinylacetamide, N-ethyl-N-vinylacetamide, N-butyl-N-vinylacetamide, N-methyl-N-vinylpropionamide, and the like; and the N-vinylpyrrolidones, such as N-vinyl-2-pyrrolidone; the amount of polymerized sulfine in the interpolymers being sufficient to assure the substantial and preferably complete water solubility of the interpolymers. Found to be particularly effective in this regard, are the interpolymers containing at least 5 mole percent and preferably from about 10 mole percent to about 99 mole percent of the sulfine in polymerized form on a theoretical monomer basis, the minimal amount of polymerized sulfine required to assure the water solubility of the interpolymers varying somewhat depending upon the particular comonomer(s) polymerized therewith.

The hereinabove described polymeric treating agents may be added directly to the dilute suspension of wood-fiber pulp that is fed to the forming wire or, more preferably, the polymer may be dissolved in water and then added to the pulp. The treating agents may be added to the pulp either before or after it is beaten or otherwise agitated, but are preferably added before or at the beater if beating is desired. Substantial improvement in the physical properties of the wood-fiber board product has been found to result irrespective of the amount of beating the pulp is given, or whether it is beaten or not. Moreover, the improvement in the properties of wood-fiber board by use of the method of this invention is substantially independent of the pH level of the pulp slurry. As hereinbefore disclosed, it has been found that the polymeric treating agents of this invention substantially increase the wet and dry strength, stiffness and stiffness retention of wood-base construction and insulation board comprised of wood-fiber pulp. Furthermore, their use in the manner described herein reduces the water retention and increases the porosity of the board in the forming operation as compared with methods heretofore known, thereby increasing production rate and production economy.

The polymeric treating agents of this invention can be produced by several different techniques. For instance, the alpha-ethylenically unsaturated sulfine represented above by Formula I can be obtained initially in monomeric form and subsequently polymerized by conventional processes for the polymerization of alpha-ethylenically unsaturated compounds either alone, so as to produce homopolymers thereof, or together with one or more comonomers hereinabove described, so as to produce interpolymers thereof. When desired initially in monomeric form, the sulfine can readily be obtained by reacting the corre-

sponding alkylthioalkyl acrylate or methacrylate represented above by Formula II with an alkylating agent, viz., dimethyl sulfate. Reactions between a thio-ether and an alkylating agent are in general discussed, for instance, in "Organic Chemistry," vol. I, 2nd ed., by H. Gilman, John Wiley and Sons, N.Y. (1948), page 867, such teachings being incorporated herein by reference. Concordant therewith, by way of illustration, the alkylation can be carried out by bringing the thio-ether and the alkylating agent into reactive admixture, in a suitable solvent or diluent if desired, and at a temperature of from about 25° C. or slightly lower, up to about 90° C. to 100° C., or slightly higher. In addition, a small amount of a conventional polymerization inhibitor, such as hydroquinone, or the like, is preferably incorporated in the reaction mixture. Moreover, the reaction is preferably carried out in a diluent which is a solvent for the thio-ether but a non-solvent for the resulting sulfine, such as benzene, isopropyl ether, etc. The sulfine product can then be separated and recovered in any convenient manner.

The polymeric treating agents of this invention can thereafter be obtained by conventional polymerization processes. Thus, for example, solution polymerization techniques can be utilized wherein an inert organic solvent solution of the sulfine alone, or in admixture with one or more comonomers, in proportions as hereinabove described, is contacted with a catalytic amount of a polymerization catalyst and maintained at a temperature at which polymerization will occur for a period of time sufficient to produce a polymer product. A particularly useful solvent which can be utilized in this connection is acetonitrile, although any other suitable inert organic solvent, such as acetone, N,N-dimethylformamide, dimethylsulfone, N,N-dimethylacetamide, ethylene carbonate, ethylene carbamate, gamma-butyrolactone, N-methyl-2-pyrrolidone, etc., can also be employed. Alternatively, bulk, suspension or emulsion polymerization techniques can also be used under otherwise similar reaction conditions, i.e., proportions, temperature, time, etc. Similarly, other diluents such as water, benzene, toluene, xylene, hexane, heptane, etc., can also be used.

The catalysts most frequently employed in the polymerization reactions, and especially in connection with solution polymerization techniques, are the free-radical-type polymerization catalysts, such as the azo compounds, of which azo-2,2'-diisobutyronitrile, dimethyl azo-2,2'-diisobutyrate, azo-2,2'-bis(2,4-dimethylvaleronitrile), azo-2,2'-diisobutyramide, and the like, are typical. Other free-radical-type polymerization catalysts which can be employed are the peroxides, such as hydrogen peroxide, acetyl peroxide, benzoyl peroxide, peracetic acid, potassium persulfate, calcium percarbonate, etc. The catalyst is ordinarily incorporated in the polymerization reaction mixture in a concentration of from about 0.01 percent to about 5 percent or more by weight, and preferably from about 0.2 to about 2 percent by weight, based upon the total weight of monomer present, although any catalytic amount thereof can be utilized.

In general, the polymerization is carried out by contacting the monomers with the catalyst at a temperature of from about -10° C., or slightly lower, to about 120° C., or slightly higher, accompanied by heating or cooling, as needed to maintain the temperature at the desired level. The reaction period to be employed will depend upon a variety of factors, such as the nature of the monomer(s), catalyst and/or diluent, the reaction temperature, etc., and can vary over a wide range. For instance, a suitable reaction period generally lies in the range of from about 1 to about 200 hours, but is not necessarily limited thereto. In addition, the polymerization can be carried out under atmospheric, superatmospheric or subatmospheric pressures, as desired.

Upon completion of the polymerization reaction, the polymer product can be recovered in any convenient manner, such as by coagulation, filtration, centrifugation, etc.

The reaction product can also be employed directly in many uses for the polymer product, obviating the recovery of the polymer per se.

In an alternative manner to the polymerization technique described above, the alkylation of the thio-ether producing the sulfine, and the polymerization of the monomer(s) can be carried out in one operation by incorporating the alkylating agent in a polymerization reaction mixture containing, as the polymerizable monomer(s), the thio-ether alone, or in admixture with at least one other member of the group of comonomers specifically defined above. In such a procedure, it is to be noted, the alkylating agent should be employed in a mole ratio of at least about 0.05:1, preferably at least about 0.1:1, and more preferably at least about 0.25:1, up to about 5:1, or higher, with regard to the thio-ether. Moreover, when another comonomer is present, the alpha-ethylenically unsaturated thio-ether should be employed in an amount sufficient to provide upon alkylation and polymerization, on a theoretical monomer basis, at least about 5 mole percent, and preferably at least about 10 mole percent of a polymerized sulfine, based upon the total amount of polymerized monomers present in the resulting polymer. Such amount is readily determined by one skilled in the art in light of this disclosure. The polymerization reaction and the recovery of the resulting polymer, when desired, is carried out as otherwise described above.

The polymeric treating agents of this invention can also be prepared by reacting the alkylating agent with an initially formed polymer, i.e., either a homopolymer of the thio-ether, or a copolymer thereof with another alpha-ethylenically unsaturated comonomer as specifically defined above, the alkylation and initial polymerization reactions being carried out as otherwise described above. In such a procedure, the alkylation is preferably carried out in solution, suitable solvents being the same as those described above in connection with the polymerization reaction. The resulting polymer product can thereafter be recovered, when desired, by coagulation, filtration, centrifugation, or in any other convenient manner.

It is preferred to add the above-described water-soluble polymers of alpha-ethylenically unsaturated sulfines to the wood-fiber pulp in combination with a suitable aldehyde and particularly preferred to add them in combination with a mixture of the aldehyde and a mineral acid. Addition of the aldehyde along with the sulfine polymer results in improved performance, i.e., the wood-fiber board produced has even greater wet and dry strength, stiffness and stiffness retention. Moreover, addition of a mineral acid plus the aldehyde plus the sulfine polymer results in even greater improvement in these properties. On the other hand, addition of aldehydes or mineral acids alone to wood-fiber pulp does not result in any significant improvement in board properties. Thus, treatment of the wood-fiber pulp with the unique combination of sulfine polymer, aldehyde and mineral acid in accordance with this invention provides properties that cannot be obtained in any other way.

The suitable aldehydes for use in this invention are compounds of the general formula:



wherein X is selected from the group consisting of a formyl radical



and an acetyl radical



m is an integer of from 1 to 3, and n is an integer of from 0 to 1. Illustrative of the suitable aldehydes one can men-

tion glyoxal, pyruvic aldehyde, succinaldehyde, glutaraldehyde, 2-hydroxyadipaldehyde, and the like.

In a preferred embodiment of the present invention, a water-soluble mineral acid is added to the wood-fiber pulp along with the sulfine polymer and the above-described aldehyde. To ensure that there is no deleterious effect on the food-fiber pulp, the mineral acid employed should preferably be a non-oxidizing mineral acid, i.e. a mineral acid which does not function as an oxidizing agent. Particularly preferred mineral acids for the purpose of this invention are hydrochloric acid, sulfuric acid, sulfurous acid and phosphoric acid.

The strength improving compositions of this invention, whether composed of sulfine polymer alone, sulfine polymer plus aldehyde, or sulfine polymer plus aldehyde plus mineral acid, are added to the wood fiber pulp in minor amounts and preferably in the form of an aqueous solution. The invention contemplates construction and insulation board comprised of wood-fiber pulp and containing from about 0.05 percent to about 5 percent, more suitably from about 0.5 percent to about 2 percent, and preferably from about 0.8 percent to about 1.2 percent, based on the weight of said pulp, of the strength improving composition. The said strength improving composition can contain 50 percent to 100 percent by weight of the normally solid, water soluble sulfine polymer hereinbefore described and 50 percent to 0 percent by weight of a mixture of an aldehyde of the formula given hereinabove and a mineral acid. Preferably, the strength improving composition is composed of 60 percent to 95 percent by weight of the sulfine polymer and 40 percent to 5 percent by weight of the mixture of aldehyde and mineral acid. The said mixture can be composed of 80 percent to 100 percent by weight of the aldehyde and 20 percent to 0 percent by weight of the mineral acid, more preferably 80 to 99 percent by weight of the aldehyde and 20 percent to 1 percent by weight of the mineral acid.

The strength improving compositions of this invention will provide enhanced properties with any of the wood-fiber pulps that are employed in the manufacture of insulation board, but are particularly effective with pulps that have not been given a high degree of chemical or mechanical refinement, e.g., groundwood, reclaimed groundwood, or "semi-chemical" pulps. The pulp should contain a substantial amount of its original lignin and/or hemicellulose content. The said strength improving compositions may be employed alone or in conjunction with other additives commonly incorporated in wood-fiber board, for example, materials functioning as sizes, waterproofing agents, fire retardants, biological control agents, and so forth.

The enhanced properties resulting from the incorporation of the strength improving compositions hereinbefore described in wood-fiber pulp employed to produce construction and insulation board can be achieved with any drying schedule normally used in the manufacture of wood-fiber board. Thus, drying can be carried out at temperatures from about 200° F., or less, to about 350° F., or more, for periods of from about 2 hours to about 100 hours. While applicant does not wish to be bound by the consequences of any theory, it is believed that chemical interaction of the additives and the woodpulp occurs during drying and that the improvement in physical properties of the product board results from such chemical interaction.

The following examples are given to illustrate the invention, it being understood that these examples are not intended to be limiting of the invention but merely illustrative thereof. In connection therewith the following definitions and descriptive material are provided.

By the term "reduced viscosity" as employed herein is meant the value obtained by dividing the specific viscosity of a polymer solution by the concentration of the

polymer in the solution, the concentration being calculated in grams of polymer per 100 milliliters of solvent at a given temperature. The specific viscosity of the polymer solution is obtained by dividing the difference between the viscosity of the polymer solution and the viscosity of the solvent by the viscosity of the solvent. The reduced viscosity of a polymer is taken as a measure of the molecular weight of the polymer, with a higher reduced viscosity indicating a higher molecular weight polymer. Conversely a lower reduced viscosity indicates a lower molecular weight polymer. In all cases, the reduced viscosity values set forth herein were determined at a concentration of 0.2 grams of polymer per 100 milliliters of solvent and at a temperature of 30° C., using a 0.5 molar aqueous sodium acetate solution as the solvent, unless otherwise specifically mentioned. As so measured, the polymeric treating agents of this invention generally have a reduced viscosity of from about 0.5 to about 5, and most frequently from about 2 to about 4. The polymers of higher molecular weight provide the greatest increase in both wet and dry tensile strengths of the wood-fiber board and are thus preferred in the practice of this invention.

Wet and dry tensile strength values reported herein were determined in accordance with methods outlined in ASTM D1037-60T, "Evaluating the Properties of Wood-Base and Particle Panel Materials." The dried board samples were brought to equilibrium under constant conditions at 23° C. and 50 percent relative humidity. Wet strength samples were first soaked for 16 hours under a 1 inch head of water at 23° C. Board density was determined in the bone-dry condition, using die-cut samples.

Stiffness measurements were made with specially constructed apparatus. In the procedure employed, die-cut strips of the insulation board, 1/2-inch wide, were cantilever mounted from plastic blocks anchored in an enclosed transparent chamber. Using the weight per unit length and thickness for each sample, the length of the cantilevered section of each piece was adjusted to apply maximum fiber stress of 2.0 pounds per square inch. The board samples were equilibrated for a 48-hour period with the test chamber in a constant temperature room held at  $25.0 \pm 0.2$ ° C. and with distilled water in the bottom of the chamber and the air within recirculated through a diffuser placed in the water. Test conditions were thus approaching water saturation at 25° C. During the equilibration period the cantilevered portion of the strip was supported in a horizontal plane by a second accurately-positioned plastic block. Deflection of the cantilevered end of the test strip was measured with a cathetometer at frequent intervals. Apparent stiffness of

the wood-fiber board was calculated using the approximate formula for the deflection of a cantilevered beam.

#### Example 1

To a ten gallon glass-lined autoclave there were charged 59.5 pounds of acetonitrile, 4.7 pounds of acrylamide, 3.1 pounds of 2-methylthioethyl acrylate, 2.7 pounds of dimethyl sulfate, and 0.2 pound of acetyl peroxide. The autoclave was purged with nitrogen and heated to 50° C. and after an induction period of about 2 hours the polymerization began as indicated by a temperature rise of about 4° C. The polymerization reaction was allowed to proceed for an additional 4 hours, after which time the autoclave was cooled and the polymer suspension dumped into a centrifuge. After washing the polymer three times with dry acetone and drying in a vacuum dryer for about 24 hours at 50° C., there were recovered, in the form of a white free flowing powder, approximately 7.2 pounds of a polymer composed of approximately 48 percent by weight of polymerized (2-acryloxyethyl)dimethylsulfonium methylsulfate and 52 percent by weight of polymerized acrylamide. This polymer had a reduced viscosity in 0.5 molar sodium bisulfite of 3.0.

In a similar manner, polymers are produced by replacing the acrylamide with vinyl acetate or N-methyl-N-vinylacetamide or N-vinyl-2-pyrrolidone or ethyl acrylate or 2-cyanoethyl acrylate.

#### Examples 2-7

A wood-fiber pulp containing 59.8 percent water as taken from the grinding mill was partially shredded by hand and then added to distilled water to form a slurry containing 1 weight percent pulp on a bone dry basis. The slurry was dispersed in a laboratory Osterizer running at top speed for a period of one minute and then 200 grams were poured into a laboratory Buchner funnel fitted with a 40 mesh stainless steel screen and a concentrically mounted glass cylinder sealed with a rubber gasket. The slurry was permitted to drain under low vacuum and then the wood-fiber pulp mat was removed from the funnel, sandwiched between stainless steel screens and pressed for 2 minutes under a 10 pound weight. The mat was then removed and baked in a forced draft oven for 16 hours at 105° C. to produce a wood-fiber board product approximately 1/8-inch thick.

Physical properties of wood-fiber board samples prepared in the above-described manner are summarized in Table I below. Where it is indicated that a strength improving composition was added to the pulp, the components of the composition were dissolved in water and then added to the pulp slurry prior to dispersion in the Osterizer.

TABLE I

| Ex. No. | Additive      | Concentration (Weight Percent) <sup>1</sup> | Board Strength       |                      | Dry Board Density (g./cc.) |
|---------|---------------|---------------------------------------------|----------------------|----------------------|----------------------------|
|         |               |                                             | Dry Tensile (p.s.i.) | Wet Tensile (p.s.i.) |                            |
| 2-----  | None-----     | None-----                                   | 19.9                 | 5.6                  | 0.1527                     |
| 3-----  | A-----        | 0.5                                         | 41.2                 | 14.5                 | 0.1623                     |
| 4-----  | A-----        | 1.0                                         | 48.7                 | 15.4                 | 0.1660                     |
| 5-----  | B-----        | 1.0                                         | 43.5                 | 8.0                  | 0.1579                     |
| 6-----  | A+Glyoxal+HCl | 1.0+0.1+0.01                                | 68.4                 | 19.4                 | 0.1749                     |
| 7-----  | A+Glyoxal+HCl | 1.0+0.5+0.05                                | 59.5                 | 17.3                 | 0.1700                     |

<sup>1</sup> Based on bone dry weight of wood pulp.

A = Polymer comprised of 10 mole percent polymerized (2-acryloxyethyl) dimethylsulfonium methylsulfate and 90 mole percent polymerized acrylamide (reduced viscosity = 3.0).

B = Polymer comprised of 25 mole percent polymerized (2-acryloxyethyl) dimethylsulfonium methylsulfate and 75 mole percent polymerized acrylamide.

Consideration of the results presented in Table I above shows that both wet- and dry-strength of the wood fiber board is greatly increased by the addition of a sulfine polymer typical of those disclosed herein and that even greater improvement in these properties results by combination of an aldehyde and a mineral acid typical of those disclosed herein with the sulfine polymer.

*Example 8*

Wood-fiber board samples were prepared in a similar manner to that described in Examples 2-6 above and wet- and dry-strength values were determined for various additives. Results are reported in Table II below.

TABLE II

| Additive        | Concentration (Weight Percent) <sup>1</sup> | Board Strength       |                      |
|-----------------|---------------------------------------------|----------------------|----------------------|
|                 |                                             | Dry Tensile (p.s.i.) | Wet Tensile (p.s.i.) |
| None            |                                             | 23.1                 | 5.63                 |
| HCl             | 0.01                                        | 19.1                 | 5.48                 |
| Glyoxal         | 0.1                                         | 21.2                 | 4.28                 |
| A + Glyoxal     | 1.0+0.1                                     | 38.9                 | 12.5                 |
| A + Glyoxal+HCl | 1.0+0.1+0.0001                              | 45.4                 | 14.4                 |

<sup>1</sup> Based on bone dry weight of wood pulp.

A = Polymer comprised of 10 mole percent polymerized (2-acryloxyethyl) dimethylsulfonium methylsulfate and 90 mole percent polymerized acrylamide (reduced viscosity = 3.0).

In this particular test series, the tensile strengths did not reach as high levels as those shown in Examples 2-7 but performance differences within the series are evident and indicate that the combination of sulfine polymer, aldehyde and mineral acid is uniquely effective in improving the tensile properties of wood-fiber board.

*Example 9*

Wood-fiber board samples were prepared in a similar manner to that described in Examples 2-7 above and stiffness values were determined in the manner hereinbefore described for various additives. Results of this series of tests are reported in Table III below.

TABLE III

| Additive        | Concentration (Weight Percent) <sup>1</sup> | Apparent Stiffness of Wood-Fiber Board (p.s.i.) |                |                |
|-----------------|---------------------------------------------|-------------------------------------------------|----------------|----------------|
|                 |                                             | Initial                                         | After One Hour | After One Week |
| None            |                                             | 1,885                                           | 311            | 107            |
| A               | 1.0                                         | 2,978                                           | 589            | 192            |
| A + Glyoxal+HCl | 1.0+0.01+0.002                              | 3,273                                           | 629            | 196            |

<sup>1</sup> Based on bone dry weight of wood pulp.

A = polymer comprised of 10 mole percent polymerized (2-acryloxyethyl) dimethylsulfonium methylsulfate and 90 mole percent polymerized acrylamide (reduced viscosity = 3.0).

Results presented in Table III above indicate that the addition of a sulfine polymer typical of those disclosed herein to wood-fiber board greatly increases its initial and apparent stiffness and that even greater improvement in this physical property is achieved by addition of an aldehyde and mineral acid typical of those disclosed herein along with the sulfine polymer.

Various changes and modifications can be made in practicing the present invention without departing from the spirit and scope thereof, and therefor it is intended to include within the scope of the appended claims all such modifications and variations as may be apparent to those skilled in the art from the description and illustrative examples given herein.

What is claimed is:

1. A wood-base construction and insulation board comprised of wood-fiber pulp and containing from about 0.05

percent to about 5 percent, based on the weight of said pulp, of a strength improving composition composed of (1) 60 percent to 95 percent by weight of a normally solid, water soluble, sulfine polymer selected from the group consisting of (a) homopolymers of an alpha-ethylenically unsaturated sulfine of the formula:



wherein R is selected from the group consisting of hydrogen and the methyl radical, R' is an alkylene radical of from 1 to 4 carbon atoms, and R'' is an alkyl radical of from 1 to 4 carbon atoms, and (b) interpolymers of said sulfine with at least one copolymerizable monomer selected from the group consisting of (i) the alkylthioalkyl-acrylates and methacrylates of the formula:



wherein R, R' and R'' are as defined above, (ii) acrylamide and methacrylamide, (iii) the alkyl and cyano-alkyl acrylates and methacrylates of the formula:



wherein R is as defined above, R''' is an alkylene radical of from 1 to 10 carbon atoms, and Y is selected from the group consisting of hydrogen and the cyano radical, (iv) the vinyl alkoanoates of the formula:



wherein R'' is as defined above, (v) the N-alkyl-N-vinyl-alkylamides of the formula:



40 wherein each R'' is independently selected as defined

above, (vi) N-vinylpyrrolidone, and (vii) vinylbenzene, said interpolymers containing in polymerized form and on a theoretical monomer basis from about 10 to about 99 mole percent of said alpha-ethylenically unsaturated sulfine, and (2) 40 percent to 5 percent by weight of a mixture of 80 to 99 percent by weight of an aldehyde of the general formula:



70 wherein X is selected from the group consisting of a formyl radical and an acetyl radical, m is an integer of from 1 to 3, and n is an integer of 0 to 1, and 20 percent to 1 percent by weight of a mineral acid selected from the group consisting of hydrochloric acid, sulfuric acid, sulfurous acid and phosphoric acid.

2. The wood-base construction and insulation board of claim 1 wherein said aldehyde is glyoxal.

3. The wood-base construction and insulation board of claim 1 wherein said mineral acid is hydrochloric acid.

4. A wood-base construction and insulation board comprised of wood-fiber pulp and containing from about 0.5 percent to about 2 percent, based on the weight of said pulp, of a strength improving composition composed of (1) 60 percent to 95 percent by weight of a normally solid, water soluble, sulfine polymer selected from the group consisting of (a) homopolymers of an alpha-ethyl-eneically unsaturated sulfine of the formula:



wherein R is selected from the group consisting of hydrogen and the methyl radical, R' is an alkylene radical of from 1 to 4 carbon atoms, and R'' is an alkyl radical of from 1 to 4 carbon atoms, and (b) interpolymers of said sulfine with at least one copolymerizable monomer selected from the group consisting of (1) the alkylthio-alkylacrylates and methacrylates of the formula:



wherein R, R' and R'' are as defined above, (ii) acrylamide and methacrylamide, (iii) the alkyl and cyanoalkyl acrylates and methacrylates of the formula:



wherein R is as defined above, R''' is an alkylene radical of from 1 to 10 carbon atoms, and Y is selected from the group consisting of hydrogen and the cyano radical, (iv) the vinyl alkanoates of the formula:



wherein R'' is as defined above, (v) the N-alkyl-N-vinyl-alkylamides of the formula:



wherein each R'' is independently selected as defined above (vi) N-vinylpyrrolidone, and (vii) vinylbenzene, said interpolymers containing in polymerized form and on a theoretical monomer basis from about 10 to about 99 mole percent of said alpha-ethyl-eneically unsaturated sulfine, and (2) 40 percent to 5 percent by weight of a mixture of 80 to 99 percent by weight glyoxal and 20 percent to 1 percent by weight hydrochloric acid.

5. A wood-base construction and insulation board comprised of wood-fiber pulp and containing from about 0.5 percent to about 2 percent, based on the weight of said pulp, of a strength improving composition composed of (1) 60 percent to 95 percent by weight of a normally solid, water soluble copolymer of (2-acryloxyethyl)dimethylsulfonium methylsulfate and acrylamide, said copolymer containing in polymerized form and on a theoretical monomer basis from about 10 to about 99 mole percent of said (2-acryloxyethyl)dimethylsulfonium methylsulfate, and (2) 40 percent to 5 percent by weight of a mixture of 80 to 99 percent by weight glyoxal and 20 to 1 percent by weight hydrochloric acid.

6. A wood-base construction and insulation board comprised of wood-fiber pulp and containing about 0.8 percent to about 1.2 percent, based on the weight of said pulp, of a strength improving composition composed of about 90 percent by weight of a normally solid, water soluble copolymer of (2-acryloxyethyl)dimethylsulfonium methylsulfate and acrylamide, said copolymer contain-

ing in polymerized form and on a theoretical monomer basis about 10 mole percent of said (2-acryloxyethyl)dimethylsulfonium methylsulfate, and about 10 percent by weight of a mixture of about 99 percent by weight glyoxal and about 1 percent by weight hydrochloric acid.

7. In a process for the production of a wood-base construction and insulation board comprised of wood-fiber pulp, the improvement which comprises applying to said wood-fiber pulp in aqueous suspension about 0.05 percent to about 5 percent, based on the weight of said pulp, of a strength improving additive composition composed of (1) 60 percent to 95 percent by weight of a normally solid, water soluble, sulfine polymer selected from the group consisting of (a) homopolymers of an alpha-ethyl-eneically unsaturated sulfine of the formula:



wherein R is selected from the group consisting of hydrogen and the methyl radical, R' is an alkylene radical of from 1 to 4 carbon atoms, and R'' is an alkyl radical of from 1 to 4 carbon atoms, and (b) interpolymers of said sulfine with at least one copolymerizable monomer selected from the group consisting of (1) the alkylthio-alkylacrylates and methacrylates of the formula:



wherein R, R' and R'' are as defined above, (ii) acrylamide and methacrylamide, (iii) the alkyl and cyanoalkyl acrylates and methacrylates of the formula:



wherein R is as defined above, R''' is an alkylene radical of from 1 to 10 carbon atoms, and Y is selected from the group consisting of hydrogen and the cyano radical, (iv) the vinyl alkanoates of the formula:



wherein R'' is as defined above, (v) the N-alkyl-N-vinyl-alkylamides of the formula:



wherein each R'' is independently selected as defined above (vi) N-vinylpyrrolidone, and (vii) vinylbenzene, said interpolymers containing in polymerized form and on a theoretical monomer basis from about 10 to about 99 mole percent of said alpha-ethyl-eneically unsaturated sulfine, and (2) 40 percent to 5 percent by weight of a mixture of 80 to 99 percent by weight of an aldehyde of the general formula:



wherein X is selected from the group consisting of a formyl radical and an acetyl radical, m is an integer of from 1 to 3, and n is an integer of from 0 to 1, and 20 percent to 1 percent by weight of a mineral acid selected from the group consisting of hydrochloric acid, sulfuric acid, sulfurous acid and phosphoric acid.

8. The process of claim 7 wherein said aldehyde is glyoxal.

9. The process of claim 7 wherein said mineral acid is hydrochloric acid.

10. In a process for the production of a wood-base construction and insulation board comprised of wood-fiber pulp, the improvement which comprises applying to said wood-fiber pulp in aqueous suspension about 0.5

13

percent to about 2 percent, based on the weight of said pulp, of a strength improving composition comprised of (1) 60 percent to 95 percent by weight of a normally solid, water soluble copolymer of (2-acryloxyethyl)dimethylsulfonium methylsulfate and acrylamide, said copolymer containing in polymerized form and on a theoretical monomer basis from about 10 to about 99 mole percent of said (2-acryloxyethyl)dimethylsulfonium methylsulfate, and (2) 40 percent to 5 percent by weight of a mixture of 80 to 99 percent by weight glyoxal and 20 to 1 percent by weight hydrochloric acid.

11. In a process for the production of a wood-base construction and insulation board comprised of wood-fiber pulp, the improvement which comprises applying to said wood-fiber pulp in aqueous suspension about 0.8 percent to about 1.2 percent, based on the weight of said pulp, of a strength improving composition composed of about

5 10 15

14

90 percent by weight of a normally solid, water soluble copolymer of (2-acryloxyethyl)dimethylsulfonium methylsulfate and acrylamide, said copolymer containing in polymerized form and on a theoretical monomer basis about 10 mole percent of said (2-acryloxyethyl)dimethylsulfonium methylsulfate, and about 10 percent by weight of a mixture of about 99 percent by weight glyoxal and about 1 percent by weight hydrochloric acid.

## References Cited

## UNITED STATES PATENTS

|           |        |                 |       |         |   |
|-----------|--------|-----------------|-------|---------|---|
| 2,285,490 | 6/1942 | Broderick       | ----- | 162—158 | X |
| 3,096,228 | 7/1963 | Day et al.      | ----- | 162—158 | X |
| 3,130,117 | 4/1964 | Humiston et al. | ----- | 162—168 |   |
| 3,207,656 | 9/1965 | Eldred et al.   | ----- | 162—168 |   |

S. LEON BASHORE, Primary Examiner.